

## UNITED STATES PATENT OFFICE

2,203,507

## LUBRICANT AND METHOD OF LUBRICATION

Theodore G. Roehner, Malverne, and Emmett S. Carmichael, Jackson Heights, N. Y., assignors to Socony-Vacuum Oil Company, Incorporated, New York, N. Y., a corporation of New York

No Drawing. Application December 11, 1937,  
Serial No. 179,256

7 Claims. (Cl. 87—9)

This invention is directed to a method of lubrication and to lubricants for use in the high speed cold rolling of strip steel and in similar circumstances. The method of lubrication used in such applications has an important bearing upon the efficiency of the steel production process as a whole and few methods of lubrication and few lubricants now available are capable of withstanding the rigorous conditions imposed to give a highly economical operation of the continuous high speed cold rolling strip steel process.

In this newly developed process of strip steel manufacture the speed of travel through the mills is relatively quite high and the rate of reduction is high in proportion to the speed. The product is used both for plating purposes such as in the production of tinned strip and a considerable amount is also used in the form of "black" sheet. The heat generated in this high speed reduction is dissipated by spraying the strip with water. Because of the large percentage of reduction at high speeds, the lubrication problem possesses the nature of a problem of extreme pressure lubrication. Because of the application of water it calls for lubricants persistent in the presence of water. Because the final use of the strip is in applications where the surface condition and/or appearance of the strip is very important, the lubricant must be capable of clean removal. As an example of the conditions to be met, mills for the high speed cold rolling of strip may handle a sheet of a width of 26" to 28" at a rate of about 1400 feet per minute while reducing it in gauge from about 0.08" to about 0.008". The strip material being rolled has been pickled prior to rolling. The heat arising from rolling is dissipated by the application of water sprays before and after rolling. Lubricant is applied to the strip material being rolled prior to each reduction in gauge, that is, the usual mill accomplishes the total reduction in gauge by passage through several sets of rolls, and the lubricant is applied prior to passage through each set of rolls, the first application of lubricant usually being immediately after the pickling operation while the sheet is being prepared for entry to the roll mill. The lubricant must discharge an extreme pressure function in that it must be capable of lubricating during reduction sufficiently to prevent seizure and marring of surfaces while at the same time it must not over lubricate to such a degree that there might be a tendency for the rolls to slip upon the strip material rather than reduce it.

An important measure of the capability of the oil to lubricate properly under these conditions is its ability to give immediate reduction to final gauge, that is, with some oils not highly capable the rate of application of reduction to strip commencing to pass through the mill may be re-

quired to be so low that the strip which passes through the mill in the first few seconds of operation is intolerably over-size. With incapable lubricants this frequently requires the clipping and rejection of 200 to 500 feet from the front end of each coil of strip which, of course, represents an economic loss. The lubricant must also be able to withstand the action of the water sprays. It must exhibit some capability for preferential wetting of heated metal in the presence of water, otherwise the sprays would remove it. Of considerable importance the lubricant must be of such a nature that it can be readily removed from the finished strip by the usual process of electrolytic washing in a slightly alkaline bath. This capability of removal is important for strip to be tinned, etc., in that it permits proper application of the coating. It is even more important in strip to be used in the "black" form, since many lubricants either by some alteration between rolling and cleaning or by incapability of being completely removed, leave quite perceptible markings upon the "black" strip.

This invention has for its object the provision of a method for lubrication and of lubricants, especially adapted for use in the cold rolling of strip in high speed mills.

A major object is the provision of a method of lubrication capable of permitting realization to the fullest extent of all of the production economies inherent in this method of steel processing.

A further object is the provision of lubricants capable of permitting rolling with substantial reduction at high speeds without either seizure, tearing, or marring of the surface of the rolled material on the one hand, or slippage of the rolls on the other.

A further object is the provision of lubricants for these purposes capable of easy, thorough and uniform application of lubricant film, capable of maintaining that film in the presence of considerable quantities of water, capable of ready removal after processing by the usual facilities available and possessed of relatively great freedom from producing stains upon the processed material under the conditions of processing.

This invention is based upon the discovery that these benefits may be obtained by applying to the steel strip in its progress through the mill, certain novel lubricants which combine the properties outlined above, which novel lubricants are made by compounding together a lubricant oil base, palm oil, and a material of the nature of an extreme pressure characterizing ingredient.

The principal ingredient in these lubricants in point of volume is the mineral oil lubricating base. Its nature is dependent upon the requirements of the particular mill or operation to which it is to be applied. It may range from a mineral

oil of medium or low viscosity through oils of the nature of cylinder stocks of high viscosity and possessed of a somewhat waxy nature for applications where a material of higher viscosity is preferred, and it may preferably consist for most typical applications of a mineral oil fraction partaking very largely of the nature of petrolatum, or a mixture of mineral oil fractions of such nature that the final compounded lubricant has a viscosity of about 150 to about 80 seconds Saybolt Universal at temperatures of from about 130° F. to about 150° F. That is, for the usual application the mineral oil base is preferably the commercial product known as petrolatum, which is an amorphous wax substantially free from crystalline structure, and which may or may not contain mineral oil. The palm oil fraction is the usual palm oil commercially supplied under the commercial designation of Niger palm oil. The extreme pressure characterizing bases may be of several of the kinds usually used in the art for such purposes. For example, they may be any of the sulphurized fatty materials. A particularly useful form is that made by sulphurizing animal fatty materials such as, for example, sulphurized sperm oil containing about 15% of sulphur. Another form of extreme pressure characterizing base which, however, should be used only in rather minor quantities is the class known as chlorinated extreme pressure bases, particularly those made by chlorinating petroleum fractions as, for example, by chlorinating a petroleum fraction of medium viscosity until it contains about 30% of chlorine by weight. To exemplify several lubricants compounded of these ingredients and capable of use under the conditions outlined, the following examples are presented:

*Example 1*

|                         | Per cent by weight |
|-------------------------|--------------------|
| Sulphurized sperm oil   | 10                 |
| Chlorinated mineral oil | 4                  |
| Niger palm oil          | 10                 |
| "Paraffin" oil          | 15                 |
| Petrolatum              | 61                 |

In the above example, the sulphurized sperm oil is one containing 15% of sulphur. The chlorinated mineral oil is an oil of medium viscosity chlorinated to contain 30% of chlorine. The paraffin oil is a light neutral oil of 100 seconds viscosity Saybolt Universal at 100° F. The petrolatum is a 122-130° F. melting point commercial grade petrolatum of Pennsylvania origin. The compounded product has a melting point of about 119° F. and exhibits the physical characteristics of a petrolatum.

*Example 2*

A more fluid product may be made with the following formula:

|                       | Per cent by weight |
|-----------------------|--------------------|
| Sulphurized sperm oil | 5                  |
| Niger palm oil        | 10                 |
| Cylinder stock        | 85                 |

In the above formula the cylinder stock is a commercial grade of cylinder stock produced as an over-head distillate from Coastal crude. The finished product is possessed of a flash of about 445° F., a pour test of about 10° F., a viscosity of 139 seconds Saybolt Universal at 210° F. and a color which is dark green or almost black.

*Example 3*

For some applications a considerably more fluid material is indicated and under such circumstances the following formula may be found useful.

|                         | Per cent by weight |
|-------------------------|--------------------|
| Sulphurized sperm oil   | 10                 |
| Chlorinated mineral oil | 4                  |
| Niger palm oil          | 10                 |
| Sulphonic acid soaps    | 35                 |
| "Paraffin" oil          | 75.65              |

With the exception of the sulphonic acid soaps the ingredients used above are as previously described. The addition of the sulphonic acid soaps is an optional feature. A small amount may be added to assist in removal of the material from the finished stock. The compounded lubricant is possessed of a pour of 15 F., a viscosity of 170 seconds Saybolt Universal at 100° F. and a viscosity of 79 seconds at 210° F.

In the above formulae it must be understood that the composition indicated by Example 1, namely, that composition which has a consistency like cup grease and is based upon the use of a mineral oil fraction of the nature of petrolatum, is the preferred type of composition. When this composition is applied to the material passing through a mill for the high speed cold rolling of strip steel at a point prior to each major reduction in gauge as herein outlined, it will be found that the mill is enabled to perform at a uniformly high degree of efficiency securing complete reduction substantially from the instant of starting a strip through the mill, securing a smoothly finished sheet free of imperfections due to seizure and similar faults and producing a finished sheet substantially free from stains and imperfections due to the nature of the lubricant. It will also be observed that with the use of this lubricant the reduction in gauge is uniform and efficient with no tendency toward slippage of the rolls without performing useful work. Additionally, the use of this lubricant, thus applied, will permit of attaining these results while securing a considerably reduced consumption of power for the production of a given amount of strip material. More fluid oils of this type as exemplified by Examples 2 and 3 do not permit of quite as good operation under the usual conditions as does the lubricant of Example 1. They do show however, that very considerable improvement over lubricants of the type formerly used which is possessed by all of the lubricants of the class herein discussed.

While certain numerical examples and data have been given herein, it is to be understood that this invention is not limited thereby or thereto, but is subject only to such limitations as are expressed in the following claims.

We claim:

1. A lubricant composition comprising in excess of 50% of a heavy mineral oil fraction, not more than about 20% of palm oil and not more than about 20% of substantially "non-corrosive" sulphur-containing extreme pressure lubricant bases.

2. A lubricant composition comprising about 10% of palm oil, about 15% of extreme pressure bases containing about 15% of sulphur, about 15% of low viscosity petroleum lubricant fraction and about 60% of petrolatum.

3. A lubricant composition comprising about 10% palm oil, about 10% of sulphurized fatty

material containing about 15% sulphur, about 4% of a chlorinated organic material containing about 30% of chlorine, about 15% of a low viscosity petroleum lubricant fraction and about 5 60% of petrolatum.

4. A lubricant composition consisting of

|                         | Per cent by weight |
|-------------------------|--------------------|
| Sulphurized sperm oil   | 10                 |
| Chlorinated mineral oil | 4                  |
| Niger palm oil          | 10                 |
| Mineral oil             | 15                 |
| Petrolatum              | 61                 |

5. A lubricant composition comprising about 10% palm oil, about 5% of sulphur-containing extreme pressure characterizing bases and a petroleum lubricant fraction of the nature of cylinder stock.

6. A lubricant composition consisting of

|                       | Per cent by weight |
|-----------------------|--------------------|
| Sulphurized sperm oil | 5                  |
| Niger palm oil        | 10                 |
| Cylinder stock        | 85                 |

7. A lubricant composition consisting of

|                         | Per cent by weight |
|-------------------------|--------------------|
| Sulphurized sperm oil   | 10                 |
| Chlorinated mineral oil | 4                  |
| Niger palm oil          | 10                 |
| Mineral oil             | 75.65              |
| Sulphonic acid soaps    | 0.35               |

THEODORE G. ROEHNERR.  
EMMETT S. CARMICHAEL.